

# United States Patent Office

2,873,223

Patented Feb. 10, 1959

1

2,873,223

## METHOD OF INCREASING THE WORK FUNCTION OF METAL PARTS FOR EXAMPLE FOR ELECTRIC DISCHARGE TUBES

Wilfrid Franz Konrad Johann Niklas, New York, N. Y., assignor, by mesne assignments, to North American Phillips Company, Inc., New York, N. Y., a corporation of Delaware

No Drawing. Application November 22, 1954  
Serial No. 470,554

Claims priority, application Netherlands December 1, 1953

1 Claim. (Cl. 148—4)

Discharge tubes frequently contain metal parts which are at low potential and other metal parts which are at higher potential and which are arranged at close proximity to one another, for example electrodes of nickel or stainless steel in a monopotential lens for television picture tubes. If, now, the field strength resulting from the existing difference in potential becomes greater than the work-function of the metal parts, unwanted scattered radiation occurs. For this reason one has looked for metallic parts having as high a work-function as possible. The work function of a material is an indication of the energy required to extract electrons therefrom. Efforts have been made to solve this problem not only by varying the chemical composition of the metals used therefor, but also by particular shaping thereof. In shaping projecting edges and collars exhibiting a so-called point action were preferably avoided. Furthermore, it has been suggested to polish the metal parts by electrolytic means. Although it has been found that polishing of the surfaces of the parts in itself raises the work function, this method suffers from the disadvantage that an oxide layer usually occurs at the surface and this results in a decreased work function.

The present invention relates to a method of increasing the work function of metal parts, for example for electric discharge tubes, which do not suffer from the above-mentioned disadvantages. The invention exhibits the characteristic that the surfaces of the metal parts are subjected to the action of ultrasonic radiation.

An explanation for the occurrence of the said effect cannot be given with certainty. It may be that the ultrasonic radiation has a micro-polishing action.

Another explanation may be that the oxide layer which may occur on the outer surface is removed by the ultrasonic radiation.

It has been found advantageous to carry out the method according to the invention in such manner that the metal parts to be treated are immersed in a liquid and that the ultrasonic radiation is produced in this bath. It is

2

preferable to utilise a liquid which cannot exert an oxidizing influence upon the surfaces of the metal parts.

Furthermore, it has been found that a still higher work-function is obtained if the metal parts, before proceeding to the ultrasonic treatment, are polished and preferably polished electrolytically.

Several applications of ultrasonic irradiation are already known. Thus, for example, it has been suggested to remove fat or dirt from surfaces under the action of such radiation. Furthermore, ultrasonic radiation has been used for coating aluminium with tin. In this case it has been suggested to keep an aluminium object in a bath of molten tin and to produce therein a field of ultrasonic radiation, the action of the ultrasonic irradiation consisting in removing the oxide layer from the aluminium.

Objects treated by the method according to the invention have been found to be very suitable for use in electric discharge tubes in which the objects have to resist high tensions, for example higher than 20 kilovolts.

### Example

Electrodes for a monopotential lens for television picture tubes were subjected to ultrasonic radiation in a bath of ethyl alcohol for several minutes. The frequency was 26,000 kc./s. and the magnetostriction core was fed with 50 watts. After this treatment and drying of the surfaces, the work-function of the electrodes was found to be approximately from 20% to 25% higher than that before the treatment.

What is claimed is:

A method of increasing the work function of the surface of a metal member, which comprises first electrolytically polishing the surface of said member adapted for use as an electrode of an electric discharge tube, and thereafter immersing said member in a non-oxidizing liquid bath and subjecting it to ultrasonic radiation while in said bath to increase the work-function of said electrode.

40

### References Cited in the file of this patent

#### UNITED STATES PATENTS

1,939,712 Mahoux ----- Dec. 19, 1933  
2,329,317 Atlee ----- Sept. 14, 1943

45

#### FOREIGN PATENTS

548,960 Great Britain ----- Oct. 30, 1942

#### OTHER REFERENCES

General Electric Review, March 1952, vol. 55, No. 2, pages 60 and 61.

Bright Future for Ultrasound by J. A. Antonevich, Bettelle Tech. Review, vol. 5, No. 4, April 1956, pages 9-13.

50